

July 24, 1934.

P. CAMESCASSE

1,967,550

PROCESS FOR PRODUCING MAGNESIUM

Filed April 14, 1930



Inventor  
P. Camescasse,  
by A. B. Foster  
his attorney.

## UNITED STATES PATENT OFFICE

1,967,550

## PROCESS FOR PRODUCING MAGNESIUM

Pierre Camescasse, Paris, France, assignor to The  
Magnesium Production Co. Ltd, London, Eng-  
land

Application April 14, 1930, Serial No. 444,236  
In Germany April 24, 1929

8 Claims. (Cl. 204—19)

The present invention relates to an improved process for the electrolytic manufacture of magnesium, in which the electrolyte consists of a mixture of magnesium chloride and potassium chloride or carnalite.

5 In the known processes of this class, measures are taken, as specified in the copending patent application, filed on the 5th of April 1929, Ser. No. 440,637, Lacell, to preliminarily dehydrate the magnesium chloride before it is placed in the electrolytic vat, and in order to prevent all improper formation of oxides during this dehydration, to add to it chloride of potassium.

10 This method is defective owing to the fact that the electrolytic bath (to which are added frequently-renewed quantities of potassium chloride and in which the magnesium chloride is alone decomposed), will after a longer or shorter period of use, come to contain an excessively large proportion of potassium chloride, and it is impossible to maintain the optimum composition of the electrolyte.

15 The present invention relates to a process for the maintenance of the electrolyte at a practically constant composition, and for assuring in good conditions the addition of the potassium chloride used to further the dehydration of the magnesium chloride.

20 The process consists essentially in the removal from the electrolytic bath, when the proportion of KCl exceeds the proper value, of a certain amount of the bath, then mixing this electrolyte with the magnesium chloride which is undergoing dehydration.

25 The said electrolyte is preferably mixed with the partly dried magnesium chloride at some stage of the drying, in which the temperature is sufficiently high to provide for an instantaneous and intimate mingling. The removed electrolyte is added to such a quantity of chloride of magnesium that when the drying is completed, there remains a mixture of substantially equimolecular proportions of magnesium chloride and potassium chloride. However, in this mixture, the proportion of  $MgCl_2$  can be as high as 10 molecules of  $MgCl_2$  to 8 molecules of KCl. The reaction will still take place, although imperfectly, as far as 10 molecules  $MgCl_2$  to 5 molecules of KCl.

30 It should be noted that when thus proceeding, the potassium chloride follows a closed cycle, and that when the manufacture is proceeding under normal conditions, no further additions of KCl are needed, except to make up for the small losses.

The process is described as follows by way of example which is given as illustrative, without limiting the invention thereto.

35 The electrolysis takes place with the use of a mixture whose proportion is kept at about 70 per cent of KCl to 30 per cent of  $MgCl_2$ . The vat is supplied with a mixture of 60 per cent of  $MgCl_2$  and 40 of KCl, which product is obtained by mixing the electrolyte taken from the vat with magnesium chloride (containing  $4H_2O$ ) in the proportion of 42 per cent of the said electrolyte to 58 of melted magnesium chloride (containing about 4 molecules of water).

40 It has further been observed by the applicant that the best results are afforded for the dehydration by using a mixture whose composition comes near that of carnalite, that is, 60 per cent of  $MgCl_2$  to 40 of KCl, and hence the operator will choose the quantities of electrolyte taken from the bath and the quantity of partly dehydrated magnesium chloride to which the same is added, so as to practically maintain this proportion.

45 The portion of the electrolyte removed from the electrolytic cell may be added during one or the other step of the dehydration or before the dehydration. It is recognized that the drying takes place preferably in successive steps, in which the magnesium chloride, hydrated to the extent of 6 molecules of water, is first melted, is then held in the molten condition until it contains 4 molecules of water, and is then completely dehydrated by a subsequent operation, employing for instance the process specified in the said copending application made by Eliza Lacell executrix of Harold George Lacell No. 440,637. These 50 three operations are designated as (a) (b) and (c) in the accompanying drawing. It is possible to operate in any of the four following manners:

55 (1) When the operator adds the mixture taken from the electrolytic vat to the magnesium chloride before the beginning of the dehydration according to the cycle  $t$  he cools and dissolves the mixture and then mixes it with the solution of magnesium chloride. Its apparent heat will be 60 lost in such a process.

65 (2) He may add the mixture taken from the electrolytic vat to the molten magnesium chloride containing six molecules of water according to the cycle  $x$  during its dehydration.

70 (3) He may, by taking certain precautions, mix it according to the cycle  $y$  with the melted chloride containing four molecules of water which is at about  $250^\circ C$ .

75 (4) According to the invention, but without 80

limitation thereto, it is found easier to add in the third dehydrating step in which there is already a mass of practically anhydrous chloride, simultaneously the magnesium chloride containing four molecules of water obtained from operation (b) and the chloride mixture taken from the electrolyte.

I claim:

1. Process of manufacture of metallic magnesium by electrolysis of a mixture of the chlorides of magnesium and potassium consisting in maintaining an electrolytic bath of said fused chlorides in an electrolytic cell, withdrawing from said cell a portion of the electrolyte rich in chloride of potassium, adding to this portion while in a hot condition and without previously adding water thereto, magnesium chloride containing some water, to serve as the primary material to be electrolyzed, heating sufficiently to dehydrate the mixture thus obtained, and returning the so dehydrated mixture into the electrolytic cell.

2. Process of electrolysis for the production of metallic magnesium, which comprises maintaining in the electrolytic cell a mixture of chlorides of magnesium and potassium, withdrawing from the electrolytic cell a portion of the electrolyte rich in chloride of potassium, partially dehydrating chloride of magnesium serving as the primary material to be electrolyzed, and adding this partially dehydrated chloride of magnesium to said portion so withdrawn, dehydrating the mixture thus obtained and returning the so dehydrated mixture to the electrolytic cell.

3. Process according to claim 2, in which the percentage of chloride of potassium in the mixture so returned is about 40%.

4. Process of manufacture of metallic magnesium by electrolysis of a mixture of chlorides of magnesium and potassium, consisting in maintaining a mixture of said chlorides in the electrolytic cell, withdrawing from said cell a portion of the electrolyte rich in chloride of potassium, simultaneously adding to said portion, partially dehydrated chloride of magnesium, melting the mixture to dehydrate the same, and returning said molten mixture into the electrolytic cell.

5. Process of manufacture of metallic magnesium by electrolysis of a mixture of the chlorides of magnesium and potassium consisting in maintaining a bath of said fused chlorides in an electrolytic cell, withdrawing from said cell a portion of the electrolyte rich in chloride of potassium, adding to this portion magnesium chloride containing some water, serving as the primary

material to be electrolyzed, to dehydrate the added magnesium chloride and form a substantially anhydrous mixture, and returning the mixture into the electrolytic cell.

6. A process of producing metallic magnesium by electrolysis of a mixture containing magnesium chloride and potassium chloride, which comprises maintaining a bath consisting essentially of said chlorides in a fused state, in an electrolytic cell, while passing an electric current through the same sufficient to cause formation of metallic magnesium from magnesium chloride in said bath, and after a time, when the relative proportion of magnesium chloride in said bath has been substantially reduced, withdrawing from said cell a portion of the electrolyte which has due to said electrolysis, become substantially enriched in potassium chloride, mixing with this portion so withdrawn, a quantity of material consisting essentially of magnesium chloride containing some water of hydration, the relative amounts of said materials so mixed being so adjusted that the heat of the mass is sufficient to substantially dehydrate the added magnesium chloride, and to form a substantially anhydrous mixture consisting essentially of the two chlorides, which mixture is then brought into said electrolytic cell for electrolysis therein.

7. Process of electrolysis for the production of metallic magnesium, which comprises maintaining in the electrolytic cell a molten substantially anhydrous mixture of chlorides of magnesium and potassium, withdrawing from the electrolytic cell a portion of the electrolyte rich in chloride of potassium, partially dehydrating chloride of magnesium serving as the primary material to be electrolyzed, and mixing this partially dehydrated chloride of magnesium with said portion of electrolyte so withdrawn while the latter is still molten, dehydrating the mixture thus obtained and returning the so dehydrated mixture to the electrolytic cell.

8. Process of manufacture of metallic magnesium by electrolysis of a fused anhydrous mixture of chlorides of magnesium and potassium, consisting in maintaining a mixture of said chlorides in the electrolytic cell, withdrawing from said cell a portion of the electrolyte rich in chloride of potassium, adding to said portion while molten, partially dehydrated chloride of magnesium, dehydrating the mixture so formed, and returning said dehydrated mixture into the electrolytic cell.

PIERRE CAMESCASSE.

55

13

60

13

65

14

70

14

75

15